

Patented May 11, 1937

2,080,017

# UNITED STATES PATENT OFFICE

2,080,017

## PHOTOGRAPHIC DEVELOPER CONTAINING AN ANTIFOGGING AGENT

Cyril J. Staud and Merle L. Dundon, Rochester,  
N. Y., assignors, by mesne assignments, to  
Eastman Kodak Company, Jersey City, N. J., a  
corporation of New Jersey

No Drawing. Application July 5, 1935,  
Serial No. 29,971

6 Claims. (Cl. 95—88)

This invention relates to photographic developers, and more particularly to photographic developers containing antifogging agents. It is known that under certain conditions, fogging occurs during the development of a photographic plate or film. Even though the developer has been properly made up, if the developing agent has become oxidized, or if the temperature rises above 70° F., or if the development is continued for an extended time, fogging is apt to occur.

We have discovered that the addition to a developer of a small amount of an iodo substituted saturated aliphatic carboxylic acid containing less than nine carbon atoms, such, for instance, as iodoacetic acid or beta-iodopropionic acid, greatly decreases the amount of fogging taking place in the developer. Preferably, the iodo-acid is added to the developer just before development. The use of these acids as anti-fogging agents has been disclosed in Patent No. 1,954,337 of Cyril J. Staud, one of the applicants in the present case.

The iodo-acid may be introduced into the developer indirectly by incorporating it in an anti-halation backing or in the light-sensitive emulsion of the photographic film or plate, or it may be added directly to the developing bath.

To illustrate the application of our invention and its effect, several examples will be given.

### Example I

Photographic plates not sensitized with any dye, were exposed behind a tri-color sensitometer with a No. 79 Wratten light filter (a bluish filter which cuts out most of the ultra-violet light of wave lengths below 360 $\mu$ ) The developer used was one for producing high contrast, and was made up as follows:

|    |                              |             |
|----|------------------------------|-------------|
| 40 | Water (about 125° F.)        | 2.0 liters  |
|    | Eton                         | 8.8 grams   |
|    | Sodium sulfite, desiccated   | 384.0 grams |
|    | Hydroquinone                 | 35.2 grams  |
| 45 | Sodium carbonate, desiccated | 192.0 grams |
|    | Potassium bromide            | 20.0 grams  |
|    | Cold water to make           | 4.0 liters  |

The plates were developed in individual trays of this developer, to which iodoacetic acid had been freshly added in the amounts of 0, 20, 50 and 200 mgm. per 100 cc. of developer. Development was carried out at 68° F. for 8 minutes, and the following results were obtained:

| 55 | Concentration of iodoacetic acid | Speed | Gamma | Fog |
|----|----------------------------------|-------|-------|-----|
|    | 0 (control)                      | 526   | 3.1   | .76 |
|    | 20 mgm.                          | 776   | 2.7   | .25 |
|    | 50 mgm.                          | 692   | 2.6   | .20 |
|    | 200 mgm.                         | 741   | 2.6   | .21 |

From this table it is evident that the presence of iodoacetic acid in the developer brings about a marked decrease in fog, accompanied by an increase in sensitivity and a slight loss in contrast. It is also apparent that in this case 20 mgm. of iodoacetic acid had practically the same effect as 200 mgm.

Fog was also decreased when the iodoacetic acid was added to the developer 1½ hours before the development.

### Example II

Spectroscopic plates sensitized to the infra-red by tricarbocyanines were hypersensitized in ammonia, exposed, and developed in the developer described above, to which iodoacetic acid had been added in amounts of 0 and 50 mgm. per 100 cc. of developer. The plates developed in the developer containing iodoacetic acid showed practically the same sensitivity as the control, but a marked decrease in fog.

### Example III

Plates not sensitized with any dye were developed for five minutes at temperatures of 51, 68 and 86° F. in the developer described above, to which iodoacetic acid had been added in amounts of 0 and 100 mgm. per 100 cc. of developer. The results obtained were as follows:

| Temperature of development<br>° F. | No iodoacetic acid in developer |       |     | 100 mgm. iodoacetic acid per 100 cc. developer |       |     |
|------------------------------------|---------------------------------|-------|-----|------------------------------------------------|-------|-----|
|                                    | Speed                           | Gamma | Fog | Speed                                          | Gamma | Fog |
| 51                                 | 676                             | .92   | .06 | 575                                            | .28   | .08 |
| 68                                 | 708                             | 2.44  | .27 | 726                                            | 1.9   | .12 |
| 86                                 | 485                             | 3.95  | .99 | 692                                            | 3.62  | .36 |

Thus it will be seen that even at abnormally high temperatures of development, the presence of the iodo-acid greatly decreases the amount of fogging taking place, while not appreciably decreasing the contrast.

### Example IV

The materials and procedure were the same as in Example I, except that beta-iodopropionic acid was used in place of iodoacetic acid. The following results were obtained:

| Concentration of beta-iodopropionic acid | Speed | Gamma | Fog |
|------------------------------------------|-------|-------|-----|
| 0 (control)                              | 525   | 3.1   | .76 |
| 20 mgm.                                  | 617   | 3.1   | .26 |
| 50 mgm.                                  | 646   | 3.25  | .26 |
| 200 mgm.                                 | 646   | 3.3   | .22 |

Here, as in Example I, there is a marked de-

crease in fog. The increase in sensitivity is not so great as in Example I, but there is no loss in contrast.

What we claim as our invention and desire to be secured by Letters Patent of the United States is:

- 5 1. A photographic developer containing an iodo substituted saturated aliphatic carboxylic acid containing less than nine carbon atoms, in an amount sufficient to decrease fogging during development.
- 10 2. A photographic developer containing iodoacetic acid in an amount sufficient to decrease fogging during development.
- 15 3. A photographic developer containing beta-

iodopropionic acid in an amount sufficient to decrease fogging during development.

4. A photographic developer containing at least 20 milligrams, per 100 cc. of developer, of an iodo substituted saturated aliphatic carboxylic acid containing less than nine carbon atoms.

5. A photographic developer containing at least 20 milligrams of iodoacetic acid per 100 cc. of developer.

6. A photographic developer containing at least 20 milligrams of beta-iodopropionic acid per 100 cc. of developer.

CYRIL J. STAUD.  
MERLE L. DUNDON.